# EUROPEAN PATENT APPLICATION

(11) **EP 3 242 299 A1**
(43) Date of publication of application: **08.11.2017**
(21) Application number: 17169789.9
(22) Date of filing: 05.05.2017
(51) Int. Cl.: H01B 1/02, C22C 9/00, C22C 9/02

(54) **ELECTRIC CONDUCTOR FOR ELECTRICAL WINDINGS, ESPECIALLY FOR CONTINUOUSLY TRANSPOSED CABLES**

(30) Priority: 06.05.2016 IT UA20163211
(71) Applicant: De Angeli Prodotti S.r.l., 35023 Bagnoli di Sopra (PD) (IT)
(72) Inventor: PERONI, Davide, I-35042 Este (PD) (IT); MAGGIOLINI, Giada, I-35036 Montegrotto Terme (PD) (IT); SARTI, Giacomo, I-35023 Bagnoli di Sopra (PD) (IT)
(74) Representative: Borsano, Corrado

(57) **Abstract**

It is described an electrical conductor for electrical windings, especially for continuously transposed cable, in copper alloy, with the base composition of the Cu-ETP and/or Cu-OF copper , in which said copper alloy contains a quantity of tin and/or magnesium, in percent between 0.010% and 0.050% in weight.

## Description

### Field of the invention

This invention refers to an electrical conductor for electrical windings, especially for continuously transposed cable.

### Description of the prior art

The continuously transposed cable (CTC), consists of a group of rectangular-section elementary electrical conductors electrically insulated among them, which are transposed to form a continuously cable that is flexible and that permits to reduce the losses compared to a single massive conductor, with the same section.

See an example of a small length of cable type CTC in figure 1.

This cable is used for electrical windings in motors, generators and transformers and is subjected, during its utilization, to repeated mechanical stresses.

Traditionally the material used for conductors is the commercially pure copper (or Cu-ETP) or commercially pure aluminium (EN AW 1370).

In case of request of higher mechanical properties a Copper-Silver alloy is used with presence of silver of 0.1% in weight.

To use a continuously transposed cable (CTC) presents several advantages compared to a single conductor: losses reduced, higher mechanical strength of the windings and in particular a greater ability to withstand the electrodynamics stresses caused by the short circuit. With a CTC the heat dissipation is better and the temperature distribution is more uniform in the entire winding.

For example the continuously transposed cables CTC used in the windings of the transformers are made up of a generally odd number of rectangular-section conductors, commonly called flat wire. The shape used for the windings of power transformers is principally the rectangular one : the principal reason is because the rectangular shape permits the use of the available space more effectively. The flat wires are generally made of copper and coated with a polymeric enamel thin layer that ensure the electrical insulation. The cable is thus composed of a plurality of flat wires each electrically insulated from the others with an enamel, intertwined with a transpositions series and, subsequently, externally insulated with paper.

The thickness of the paper and the number of the layers used depend on the type of the application, and have the main purpose to increase the electrical insulation between winding turns, giving a certain dielectric strength. In addition to the electrical insulation, the paper wrapped in helical way allows to keep the conductor compact during the winding stages on the coil, transport and unwinding.

If there is no need for particular insulation between winding turns, the CTC cable can be without paper and wrapped only with a polyester wire or tape, resistant to transformer oil and which keeps the cable close, with the advantage of better cooling.

It is known that the higher is the conductors area, the higher will be the eddy currents losses, and is just to overcome this problem that it is usual to put in parallel more flat wires, dividing the total conductive area in a plurality of smaller conductors. To reduce the collateral effects caused by shift current and to obtain a more compact and flexible conductor, the position of the flat wires in the cable cross section is intertwined repeatedly throughout the total length of the transposed cable. Each flat wire thus assumes every possible position in the entire section of the conductor and the order of the layers in the cross section repeats cyclically. The transposition of the flat wires at regular intervals, forms a sort of rectangular cord and, furthermore, increases the flexibility of the cable itself. The periodic transposition of every flat wire on its transversal section of the cable has the advantage to keep the losses low, due to eddy currents; in this way the transformer efficiency increases, and it avoids localized high temperatures that can cause overheating and damages to the winding insulation.

Generally, a high voltage transformer is designed to last for 30-40 years. During this time a transformer could be subjected to electrical, mechanical and thermal stresses due to the working of the transmission electrical grid. In recent years, new stresses with new distribution patterns have also become more and more frequent. For example, wind and solar fields produce an increase in current that crosses the lines, generating additional loads for power transformers. In addition, energy distribution systems, including new renewable sources, increase the number of operations on the power grid such as ignition, power off and power reversal. In addition to this, there are also mechanical stresses that weaken the transformer structure and its ability to withstand short circuits.

Mechanical stresses are caused by internal forces between flat wires and cables resulting from short circuits, thermal stresses and local overheatings and overloads of currents or for cooling malfunction. Dielectric stresses are due to system overvoltage, transitory pulses or internal resonance between windings.

One of the most critical situations is caused by external short circuits that produce high currents in the transformer windings and therefore high internal electrodynamics forces in the windings.

Generally, the transformers are designed to stand the maximum peak of the three-phase current short circuit, calculated as if the transformers had been connected to an infinite bar.

The forces generated by the currents that flow in the windings are of compression for both windings, and can reach high values, so they are dangerous for the mechanical integrity of the windings during the short circuit transitory.

Radial forces are dominant due to the axial direction of the main stream and cause a number of problems such as forced deformation, conductor flexion, instability and increased diameter for external windings. This huge current undergoes winding at tremendous mechanical effort.

From the mechanical point of view, the CTC cable must have certain characteristics in terms of conductivity and mechanical strength to resist the stresses mentioned above.

From the point of view of the quantities produced and consumed worldwide, the type of material most used for these conductors is copper, in particular the Cu-ETP type (Electrolytic Tough Pitch). The Cu-ETP copper is obtained from electrolytic refining and characterized by oxygen presence and phosphorus absence.

The copper is widely used for its electrical conductivity, second only to silver and considerably influenced from the impurities. The copper electrical conductivity at 20°C is conventionally considered equal to 58.00 m/Ωmm2. This value is assumed as unit of measure of the commercial copper electrical conductivity, so this conductivity corresponds to 100% IACS (International Annealed Copper Sample) at 20°C. For high purity copper higher values could be reached, with a maximum theoretical limit of 103.5% IACS, corresponding to 60.00 m/Ωmm2 ; in any case, the standards stipulate that copper intended for electrical uses should not have electrical conductivity below 100% IACS.

To withstand the stresses, however, also the mechanical properties of the material (breaking load and proof stress) are important. For this reason the copper can be used with different levels of hardening: the higher is the hardening, the better are the mechanical properties. However, the hardening decreases the electrical conductivity even if considerably less than the impurities: the maximum impact on a commercial copper can lead to a fall of approximately 3% of the conductivity compared to the copper.

The cast copper (said wire rod) shows up generally in the annealed physical state and so it has low mechanical properties, with values of proof stress that can decrease up to 60 MPa. For increasing its mechanical properties the plastic deformation could be used, so, in this way, the hardened copper (said raw copper) can reach values of proof stress up to and over 350 MPa. Often intermediate conditions are considered, known as CPR (Controlled PRoof stress).

Figure 2 shows graphs of mechanical tension or stress σ as a function of the deformation ε for different types of copper at different levels of strength: annealed copper , raw copper, and copper at intermediate states of hardening CPR1, CPR2.

The normal CTCs flat wires production process limits the maximum hardening of the copper usable for the enamelling that happens with thermal polymerization process in ovens heated at high temperature. Indeed it is a direct proportionality that relations the level of hardening with the annealing speed, at the same temperature (the annealing is a thermal treatment that leads to a regeneration of the crystal structure hardened from cold plastic processing such as extrusion and lamination, as well as a general stress relief of the piece). For this reason the maximum level of hardening obtainable, said CPR3, corresponds to values of proof stress from 220 to 260 MPa.

The tables in figure 3 and 4, taken from BS 1432-87 norm, show respectively the hardening levels used for the production of a transposed cable and the relation between hardening state and electrical conductivity of the conductor, for cables CTC and hardening levels CPR1, CPR2, CPR3.

The hardening level CPR3 is nevertheless a limit in the final utilization of the cable CTC. Indeed the generated heat during the operational life of electrical transformers, that can leads to operational temperature up to 120°C, causes the same effects of the annealing of the copper (lower mechanical strength , hardness, etc.) though with minor speeds and with times equivalently longer (over the decades this aspect for the copper is already observable from 100 C).

To overcome these limits it is necessary that the copper electrical conductor does not have to lose too much of its mechanical characteristics with the temperature.

To avoid this annealing during operational life, it is now actually used the CuAg0.1 alloy (CW013A for the EN 1977 norm), where 0.1 stands for the percent of silver weight in the copper. Due to the electronic nature of the current flow in the metallic materials, it is evident that the impurities works as obstacles to the movement of the electronic stream itself.

The silver, however, is an optimal conductor and affects minimally the electrical conductivity of the copper, allowing to keep it at 100% IACS, ensuring to the alloy, at the same time, a higher recrystallization temperature acting on the impact of the annealing on the crystal structure.

Thanks to this CuAg0.1 alloy, it is possible to produce and utilize in the transformers a copper transposed cable with higher hardening than CPR3, with Rp0,2% more than 300 MPa. These are, for example, used in power transformers in the range from 50 up to and over 800 MVA.

However, despite the small quantities of silver in the alloy, the cost of the cable increase considerably.

So then the need arises to find copper alloys for continuously transposed cables at least as good as the one already known, but with considerably lower costs.

### Summary of the Invention

Therefore, the purpose of the present invention is to provide an electric conductor for electric windings, especially for continuous transposed cable, which eliminates the previously mentioned drawbacks and which has the required physical and mechanical characteristics.

An aim of the invention is therefore to propose a cheaper but equally valid alternative to the CuAg alloy for the CTC cable described above.

The present invention refers to an electrical conductor of the CTC continuous transposed type whose elementary conductors are made up of copper by the addition of very low concentrations of binders (concentration <0.05%), in particular copper alloy with tin and / or magnesium, such as to confer greater resistance to annealing at the temperatures of use compared to Cu-ETP.

This alloy compared with the well-known conductor alloy of copper-silver has a lower cost with the same mechanical characteristics.

It is known to use in the railway sector alloys for the contact wire (trolley). In this industry, copper alloys containing silver, tin, magnesium and cadmium (which is no longer used because it is forbidden by the latest ROHS for reasons safety) are used to improve mechanical performance and temperature resistance (creep).

These alloys, however, are mainly designed to obtain significant breaking load increments and therefore contain significant amounts of alloy elements that go to the detriment of the electrical conductivity of copper, which is one of the fundamental requirements for the use of the transposed cable.

The object of the present invention, in accordance with claim 1, is an electrical conductor for electrical windings, especially for continuously transposed cable, made of copper alloy, with the basic composition of the Cu-ETP copper and / or Cu-OF copper, characterized in that said copper alloy contains a quantity of tin and / or Magnesium, in a percentage ranging from 0.010% to 0.050% by weight.

It's also an object of the present invention, a continuously transposed cable CTC comprising a plurality of stacked parallel electrical conductors with rectangular cross-section, each electrical conductor as defined in the preceding paragraph.

It's a particular object of the present invention an electrical conductor for electrical windings, especially for continuously transposed cable, as better described in the claims which form an integral part of this description.

### Brief description of the figures

Further characteristics and advantages of the invention will become more clear from the description of preferred but not exclusive embodiments of the conductor according to the invention, with reference to the accompanying drawings, in which:
Figure 1 shows an example of a portion of the continuously transposed cable CTC;
Figure 2 shows trend graphs of mechanical tension or stress σ as a function of deformation ε for different types of copper at different levels of hardening;
Figures 3 and 4 show tables coming from BS 1432-87 standard, which illustrate respectively the hardening conditions used for the production of a transposed cable and the relationship between the level of hardening and the conductivity of the conductor for CTC cables for the following hardening states: CPR1, CPR2, CPR3;
Figure 5 shows a graph of the Proof Stress (MPa) in time of standard copper (Cu-ETP) relative to copper alloy CuSn and / or CuMg according to the invention, subjected to accelerated aging treatment to simulate working life conditions.

### Detailed Description of the preferred embodiments

The present invention refers to an electrical cable of the continuously transposed CTC type, in which elementary conductors are made of copper with addition of binders at very low concentrations (concentration < 0.05%), in particular in Copper- Tin alloy and/or copper - magnesium alloy. The influence of these binders (tin and/or magnesium) on the annealing and on recrystallization is due to the fact that they act as an obstacle for the mobility of the atoms, so that a bigger energy provision (bigger activation energy) is necessary for starting the solid state transformation, such as the recrystallization.

To address the problem of loss of conductivity, it has directed towards the low alloy content which for low concentrations leads to a loss of conductivity directly proportional to the percentage by weight.

It has been fundamental to find the optimum percent of Tin and Magnesium in the copper, to maintain high the electrical conductivity (≥100% IACS) so as to be able to fulfill the conductor function for power transformers, and at the same time it has been verified that, for these low quantities in weight of Tin and magnesium, the influence of the addition of the element permits an increase of the recrystallization temperature.

It has been found an electrical conductor for electrical windings, especially for continuously transposed cable, made of conductive material in copper alloy, with the base composition of Cu-ETP copper following the standard EN 1977, but characterized in that said copper alloy contains a defined quantity of tin, in percent between 0.010% and 0.050% in weight, preferably between 0.020% and 0.040%. A specific preferred value could be 0.025%.

It has been found, furthermore, an electrical conductor for electrical windings, especially for continuously transposed cable, made of conductive material in copper alloy, with the base composition of Cu-ETP copper following the standard EN 1977, but characterized in that said copper contains a defined quantity of magnesium, in percent between 0.010% and 0.050% in weight, preferably between 0.020% and 0.040%. A specific preferred value could be 0.030%.

It has been found also, an electrical conductor for electrical windings, especially for continuously transposed cable, made of conductive material in copper alloy, with the base composition of Cu-ETP copper following the standard EN 1977, but characterized in that said copper is of the type copper-tin-magnesium with a total percent of the elements (Tin+Magnesium) between 0.010% and 0.050% in weight, preferably between 0.020% and 0.040%. A specific preferred value could be 0.030%.

Alternatively, the copper base composition may be in accordance with the same EN 1977 standard as regards the oxygen percentage, which can be defined with the acronym "copper Cu-OF" (Oxygen Free), so as, as stipulated by the standard, to comply with the requirements of hydrogen embrittlment.

It is also possible that the base composition of the copper satisfy both the 2, 2, 4above defined requirements Cu-ETP and Cu-OF.

The graph in the figure 5 represents the behavior of the proof stress (Proof Stress, MPa) during the time, of the standard copper (Cu-ETP) compared to copper alloyed CuSn and/or CuMg according with the invention, submitted to accelerate aging treatment to simulate the life conditions during work. It can be seen as the standard copper suffers a decrease of the mechanical properties and how the new copper- tin, despite it is more hardened, maintains them approximately constants, at the same treatment temperature, confirming the purpose of better behavior of the standard alloys in thermal stress conditions.

This higher resistance to annealing and recrystallization permits to pass the enameling phase and the transformer life phase without significant losses of mechanical properties even in case of very high hardening.

Thanks to this increased annealing resistance with the new developed alloys is thus possible to produce (enameling) and utilize in the transformers a copper transposed cable with hardening higher than CPR3, with Rp0,2% even higher than 300 MPa, like the CuAg0.1 alloy, but without the drawback of the high cost of the material. as far as the cost is concerned, the CuSn and CuMg alloys permits a remarkable saving compared to the silver alloy: this fact plays an important role in the present invention, since it proposes a cheaper alternative to an already established fabrication technology in CTC field.

It is to be noted that the standard for the cast copper (wire rod) Cu-ETP admits as impurities very little quantities of Sn or Mg, the presence of which is thus casual and not guaranteed, while in the present invention the addition of Sn and Mg is done intentionally and maintained in a specific range.

The presence of very little quantities of impurities (for example of Sn and Mg but also other elements) comes from production process of copper Cu-ETP that provide for the refining of the copper, starting from an initial condition with presence of these impurities, and it has the purpose to eliminate indistinctly all said impurities in the starting mineral, to obtain in the end a "commercially pure" copper. According to the starting mineral, different concentrations of impurities can be present , even also Sn and Mg, but this concentrations are quite random.

For the production of the conductor of the present invention, it is necessary to proceed with the copper refining first, and then adjusting the concentration of the alloy elements following the percentage described above.

However, the production process of the material of the present invention could happen following a known method: instead of silver, the above described quantities of tin and/or magnesium are added.

Object of the present invention is thus an electrical conductor for electrical windings, especially for continuously transposed cable CTC, made of copper alloy in the variants above described with presence of tin and/or magnesium with the above weight percent.

Object of the present invention is also a continuously transposed cable CTC, made of a plurality of stacked parallel electrical conductors of rectangular section (flat wire), each one made of that copper alloy in the variants above described with presence of tin and/or magnesium with the above weight percent.

Also the production process of the continuously transposed cable CTC of the present invention can be made with a known method: instead of the copper alloy with silver, for each of the conductors it is used a copper alloy with tin and/or magnesium, with the mentioned percent weight quantities.

The conductor, object of the present invention, is thus suitable for the use in electrical transformers in oil, resin, or dried.

For this purpose it is particularly useful the rectangular-shaped section of the flat wire of the conductor, because it is easily foldable to build the transformer windings. The rectangular shape optimizes also the spatial occupation, minimizing the empty areas.

The conductor, object of the invention, could be insulated through the surface application of paper (for example cellulose) and/or with enamel, or wrapped with paper and/or with wire and/or with net and/or with polymeric tapes. All said insulators are of a known type.

The conductor, object of the invention, shows a proof stress Rp0,2% between 100 MPa and 400 MPa, preferably between 200 MPa and 400 MPa, thus it comprises all the usable known hardening levels.

Embodiments variants are possible to the non-limiting example described, without departing from the scope of the present invention, including all equivalent realizations for a skilled technician.

The elements and the characteristics described in the different preferred forms of embodiment could be combined between them without departing from the scope of the present invention.

From the description above reported the skilled technician is able to realize the object of the invention without introducing further constructive details.

## Claims

1. Electric conductor for electric windings, especially for continuously transposed cable, made of copper alloy having the basic composition of Cu-ETP copper and/or Cu-OF copper,
**characterized in that** said copper alloy contains a percent quantity of tin and/or magnesium of 0.010% to 0.050% in weight.

2. Conductor according to claim 1, **characterized in that** said copper alloy contains a percent quantity of tin alone of 0.010% to 0.050%, preferably 0.020% to 0.040%, in weight.

3. Conductor according to claim 1, **characterized in that** said copper alloy contains a percent quantity of magnesium alone of 0.010% to 0.050%, preferably 0.020% to 0.040%, in weight.

4. Conductor according to claim 1, **characterized in that** said copper alloy contains a quantity of tin and magnesium, with a total percentage of tin and magnesium of 0.010% to 0.050%, preferably 0.020% to 0.040%, in weight.

5. Conductor according to any one of the preceding claims, comprising surface insulation provided by one or more of the following insulators: paper and/or enamel, wrapping with paper and/or thread and/or net and/or polymeric tape.

6. Conductor according to any one of the preceding claims, **characterized by** an Rp0.2% yield strength of 100 MPa to 400MPa, preferably 200 MPa to 400 MPa.

7. Continuously transposed cable CTC comprising a plurality of stacked parallel electric conductors having a rectangular cross-section, wherein each electric conductor is as claimed in any one of the preceding claims.
